

May 19, 1925.

1,538,816

F. E. IVES

COLOR PHOTOGRAPH OR FILM AND METHOD OF PRODUCING SAME

Filed Feb. 15, 1923



INVENTOR  
Frederic E. Ives,  
BY  
Rogers, Kennedy & Campbell  
ATTORNEYS.

## UNITED STATES PATENT OFFICE.

FREDERIC E. IVES, OF PHILADELPHIA, PENNSYLVANIA.

## COLOR PHOTOGRAPH OR FILM AND METHOD OF PRODUCING SAME.

Application filed February 15, 1923. Serial No. 619,187.

*To all whom it may concern:*

Be it known that I, FREDERIC EUGENE IVES, a citizen of the United States, residing at Philadelphia, in the county of Philadelphia and State of Pennsylvania, have invented a certain new and useful Color Photograph or Film and Method of Producing Same, of which the following is a specification, reference being had therein to the accompanying drawing.

This invention relates to color photographs or films and method of producing same. The invention involves both the arts of color photography and motion pictures and constitutes an improvement in both arts.

In its broad aspect the object of the invention is to afford a simple, effective and convenient mode of producing a multicolor picture or print, and one which will be less complicated and quicker to carry out and yield a better product. More particularly, an object is to produce two, by which I mean at least two, differently colored images, to be successively produced and blended in the same member or carrier, thus obviating the necessity of attaching independently produced members. It is an advantage of the present invention that the images may be produced within the body of a single colloid layer, which is the plan referred to in my prior Patents Nos. 1,175,540 of February 8th, 1916, and 1,278,668 of September 10th, 1918. The present invention improves and quickens the process of said prior patents and affords a superior resulting product. These are some of the advantages and objects of the present invention, and further objects and advantages will be elucidated in the hereinafter following description or will be apparent to those skilled in the art.

To the attainment of the above referred to objects and advantages the present invention consists in the novel processes, steps and products hereinafter described. First will be described one or more embodiments of the invention, and thereafter the novel features will be pointed out in the claims.

Two or more simultaneously exposed views or series of views will be supposed to have been taken from substantially a single viewpoint for the purpose of securing color selection negatives from which afterward

the positives or diapositives are to be made. The two-color system will be supposed to be employed, for, although the three-color system might be used, the two-color is eminently more simple and is sufficiently satisfactory for general practical purposes.

In exposing for the view or series of views constituting the subject, there may be a red screen interposed in the path of the light rays or in some other way a selection of the red rays made, and in connection therewith, a film sensitized especially for red rays may be employed. Thus red-selection negatives are obtained. Similarly a green screen and green sensitive film may be employed for securing green-selection negatives.

In my said prior Patent No. 1,278,668 the first exposure was made through the transparent celluloid base of the receiving print member from the green-representing negative, thus producing a silver image at the interior side of the gelatin layer which afterwards was toned to a red color; and, subsequently, from the red-representing negative the second printing was performed at the exterior surface of the gelatin for producing a blue-to-green image. One of the negatives, the first one, was a reversed negative so that the two images, printed from opposite sides, would properly register. After the formation of the first or interior image, the gelatin layer was required to be resensitized for the printing of the second image. It was resensitized by the iron process, giving eventually the blue-to-green image desired. The color toning of the first image was described as following the production of the second image. This process while efficient and giving good results was somewhat slow and therefore disadvantageous from a practical standpoint. Especially it was slow in regard to the steps of resensitizing and producing the second or exterior image. The present invention gives a much quicker and more satisfactory procedure.

The present invention in part may be illustrated by diagrams. In the accompanying drawings showing one mode of employing the principles of the present invention, Fig. 1 may be considered a side elevation of a red-representing negative facing downward.

Fig. 2 is a similar view of a green-representing negative facing downward.

Fig. 3 represents a sensitized colloid film facing upward and on which the final picture is to be produced.

Fig. 4 illustrates the step of printing from the red-representing negative upon the film.

Fig. 5 on an enlarged scale is a sectional view of the film or print after the production of the first image.

Fig. 6 is an elevation showing the step of printing from the green-representing negative to form the second image in the film.

Fig. 7 is an enlarged section showing the final print or picture containing both images.

Fig. 8 is a modification showing the two images both printed in the same face and level at the outer surface of the colloid layer, from negatives not reversed with respect to each other.

Fig. 9 is another modification showing the two images both printed in the same face and level at the inner surface of the colloid layer, from negatives not reversed with respect to each other.

The present invention may be conveniently carried out in the manner which will now be specifically described. Assuming the two-color system, we commence with a set of color selection negatives 10 and 11. The first negative 10 may, for example, represent the red components of the picture and the negative 11 the green components. Eventually the final picture will include a blue-to-green positive image from the first or red-representing negative, and a red image from the green-representing negative.

The print or film 12 in which the positive images are to be formed and blended comprises colloid portions 13 supported preferably on a transparent or celluloid carrier 14. The first step in the process is to expose by means of the first negative and form an image at one surface of the colloid portion of the print or film member 12. It is to be assumed that the colloid layer 13 is sensitized with silver haloid. The first printing is preferably by the red-representing negative 10, and, as shown in Fig. 4, this negative may be a reversed negative and used in such a way as to effect the exposure at the rear or through the carrier 14, so that the resulting image will be confined largely to that side of the gelatin layer which is next to its carrier, and may be referred to as the bottom or interior surface; but this exposure may alternatively be made upon the outer face, as later described.

Having been exposed, the silver image may be developed and will be found to extend into the exposed surface of the gelatin in a manner that will be roughly understood from the enlarged cross-section, Fig. 5, in which the colloid layer 13 is shown as hav-

ing a silver image 15 at its bottom side with a mass of gelatin 16 filled with silver bromid extending between the image and the top surface.

The general plan of the present improvement is to first produce an image 15 from the red-representing negative, as already stated, and then convert it to a blue-to-green image by any suitable steps such as those hereinafter described. This is contrary to said prior Patent 1,278,668 wherein the first image is produced from the green-representing negative and converted to a red colored positive. The next step of the present invention is to convert or reconvert the silver ferrocyanid base of the converted blue print to silver bromid instead of dissolving it out or making it inert to light and development as has previously been proposed. When the first or blue-to-green image is produced by the iron toning or converting process a base of silver ferrocyanid remains, and hereinafter will be specifically described how this may be converted to silver bromid. The next operation is the production of the second image by the use of the green-representing negative. The image is printed in the sensitive silver bromid, and upon development gives normal graduations of density. Fig. 6 shows this printing at the top or outer side, and Fig. 7 shows the second image 17 at the top surface of the gelatin; but it may alternatively be printed in the same face as the blue image, as later described. Finally this second image is to be toned or converted to a red color, thus completing the process.

The novel method thus described in general outline is found to be capable of quite perfectly overcoming the various recited objections and other objections that have rendered of little or no practical value the prior attempts of others. The above outline of the present process is itself insufficient to secure the best results without a more detailed description and, therefore, there will now be recited a complete specification of a practical process.

Assuming two-color cinematograph films are to be made by this invention, we may start with relatively reversed negatives 10 and 11 such as made by the method of my United States Patent No. 1,320,760, of November 4, 1919, and the final pictures 12 may be produced on ordinary standard cinematograph positive film.

First, the red-representing negative 10 may be used to print through the carrier 14 of the print or film 12, as shown in Fig. 4, as already stated. The exposed film 12 is developed by ordinary means, such as the well known monomethylparramidophenol sulfate (metol) developer, but I prefer to use a dilute developer, without bromid, with time limit to make the image thin and delineated. It should be a very fully exposed,

though thin and delicate image. One minute washing should follow. The print may then be immersed for two minutes in:

*Solution A.*

|              |     |       |
|--------------|-----|-------|
| Water        | 460 | c. c. |
| Formaldehyde | 8   |       |

10 After washing for a few minutes in water the print should be immersed in the following blue or iron toning solution:

*Solution B.*

|                             |      |        |
|-----------------------------|------|--------|
| 15 Water                    | 460  | c. c.  |
| Oxalic acid                 | 3.24 | grams. |
| Potassium ferricyanid       | 1    | gram.  |
| Ferric chlorid solution, U. |      |        |
| 20 S. P.                    | 16   | c. c.  |

The print is to stay in this solution until the action is seen to be complete by examination of the deepest shadows by reflected light at the back. It requires from two to 25 five minutes, and can be carried out in white light, though I prefer to work in a bright yellow safe light. If a more prolonged immersion is given it creates a difficulty, namely a selective hardening of the gelatin, 30 which action tends to spread toward the outer surface. Such hardening might impair the production of the second or red image herein. It is found to be irregular, occurring more substantially above the 35 denser places, but it is rendered inappreciable by the use of the described quick toning action, which also minimizes other objections, without detriment to the color of the blue-to-green image. Immediate and 40 thorough washing after the toning further minimizes any tendency to selective hardening.

After such conversion of the first silver image to a cyanotype image, and after 45 thorough washing, the silver ferrocyanid base of the blue print will have its sensitiveness to light restored by conversion to silver bromid. For this purpose the print may be immersed for thirty minutes or 50 longer in a suitable halogen or bromine bath such as the following:

*Solution C.*

|                   |     |        |
|-------------------|-----|--------|
| 55 Water          | 460 | c. c.  |
| Sodium chlorid    | 1.3 | grams. |
| Potassium bromid  | 4   | grams. |
| Hydrochloric acid | 7   | c. c.  |

60 The sodium chlorid and hydrochloric acid contents of this bath can be omitted if the potassium bromid content is sufficiently increased, and sulphuric or other acid, in smaller quantity, can be substituted for hydrochloric acid. It is also desirable to

greatly decrease the light-sensitiveness of the silver bromid content of the layer, so that it approximates that of so-called gas-light paper. This permits of carrying out the operations of drying and handling in a 70 very bright and comfortable yellow light, but yet to make the prints from the green representing negative by exposures of a small fraction of a second to a 50 watt nitrogen lamp. This decrease of sensitiveness 75 is best effected by a so-called desensitizer, such as phenosaffranin, which may be added to the bromid bath. To best utilize the advantages named and at the time reduce the time of immersion necessary in the re-sensitizing bath, the following may be substituted for solution C given above:

*Solution CC.*

|                  |     |         |
|------------------|-----|---------|
| Water            | 11  | litres. |
| Potassium bromid | 450 | grams.  |
| Sulphuric acid   | 7   | c. c.   |
| Phenosaffranin   | 1   | gram.   |

Ten to fifteen minutes' immersion in this 90 bath, with occasional agitation, is sufficient. The reduction of sensitiveness by the action of phenosaffranin is much less than otherwise when it is added to the acid bromid bath, but sufficient to make its use very ad- 95 vantageous.

During baths C or CC, and subsequent operations, the film must be protected from actinic light. The bath acts to convert the silver ferrocyanid base of the blue print to 100 silver bromid, thus restoring the original silver bromid content of the colloid layer. The bath further eliminates the effects of the previous exposure to light, and equalizes the sensitiveness of all the contained silver 105 bromid. The print should next be thoroughly washed in running water. It should then be dried, for example by hanging in a dry dark room.

The resensitized print may next be exposed beneath the green-representing negative 111, as in Fig. 6. The negative should be exactly registered upon the blue image. When done visually, a green safe light is better and gives less difficulty than a red 115 or orange one; but this and other mechanical steps may be performed automatically by suitable appliances.

After the second exposure follows a second development. This development should 120 be timed, and need seldom exceed one minute with a normal developer. A "stop bath" of water containing a little acetic acid can be advantageously used following the development. Quick action of the developer, followed by the use of an acid stop bath, avoids injurious effects upon the first image. The blue image may disappear during development but gradually redevelops 125 color and intensity in the subsequent opera-

tions of fixing and washing if the second development has not been injuriously prolonged.

There are now two images, the first blue-to-green, converted from a silver image, and the second silver image awaiting conversion to red. By red is meant any sort of red, as conditions may require, including an orange red, or yellow-to-red dichroic image 10 as heretofore proposed by me for this purpose, see my U. S. Patent No. 1,376,940 of May 3, 1921. Many well known toning and converting processes may be used to produce the red color in the second or exterior image. 15 For example, I may use a copper toning process, such as suggested for the first image in said Patent No. 1,278,668 but the bath may be made up of the following:

20 *Solution D.*

|                            |            |
|----------------------------|------------|
| Water                      | 1000 c. c. |
| Cupric sulfate             | 7 grams.   |
| Potassium citrate, neutral | 28 grams.  |

25 *Solution E.*

|                            |            |
|----------------------------|------------|
| Water                      | 1000 c. c. |
| Potassium ferricyanid      | 6 grams.   |
| Potassium citrate, neutral | 28 grams.  |

30 Solutions D and E should be mixed in equal parts for the toning bath. A drop of acetic acid may be advisable, as the bath should be strictly neutral or slightly acid. A few minutes suffices to tone the second 35 silver image to a copper red color.

Preferably the copper red color is 40 strengthened or modified by dye to give the desired tone of red or red-to-yellow, in accordance with my U. S. Patents Nos. 1,300,616 granted April 15, 1919, and 1,376,940 granted May 3, 1921. The copper image is capable of selectively mordanting certain dyes, available for this purpose. For example, the copper toned image after washing, 45 may be immersed in the following:

*Solution F.*

|                          |            |
|--------------------------|------------|
| Water                    | 1000 c. c. |
| Phenosaffranin (red dye) | 1 gram.    |
| Auramine (yellow dye)    | 2 grams.   |
| Acetic acid              | 15 c. c.   |

In this solution phenosaffranin equals diamidophenylphenazonium chlorid, and auramine equals amidotetramethyldiamidodiphenylmethane hydrochlorid.

60 In lieu of this bath it is sometimes advantageous to dye first in a red bath, and then in a yellow one until the yellow color replaces the red in the lighter shades, after which washing clears all dye out of the white parts of the picture, and after drying the product is finished. In any case the depth of color should be regulated to co-ordinate with the blue image already produced, and this is 65 satisfactorily done by attention to the

strength of the dye bath, time of immersion, and amount of subsequent washing.

A quicker and cheaper method of converting the second color image to red consists in 70 converting the silver image to silver ferricyanid, which also mordants basic red and yellow dyes, and it is even practicable to accomplish this in a single combined bath of potassium ferricyanid, chromic acid and certain basic dyes. For example, if, to a 75 bath of phenosaffranin containing 1 part in 4,000 of water, is added as much of a solution of equal parts of potassium ferricyanid and chromic acid as can be stirred into it without producing much permanent precipitate, and then filtered, it will very slowly 80 convert the silver image to a red image, which in course of time becomes brilliant and transparent, and can be modified in hue by subsequent immersion in a bath of 85 auramin. This method is particularly sensitive to the presence of any trace of the sodium thiosulphate used in fixing the second silver print, which should therefore be very thoroughly washed in running water, and in 90 the case of motion picture film, it should be wound on a frame which has never been touched by the hypo solution before immersing in the dye bath.

A very important feature of the process 95 set forth, which differentiates it from all processes heretofore proposed for producing two colored images in a single colloid layer, both in silver bromid, by exposure and development to metallic silver, and subsequent 100 conversion to color images, is that in my process the second print is not limited to an uneven residual layer of silver bromid, but is made in a fully and evenly charged layer of silver bromid, and also in the presence 105 of an image transparent to actinic light, so that the second print can be made upon either face of the sensitive layer, and extend to any depth within it. It becomes possible 110 not only to make both images in the same face and level of the colloid layer, in contradistinction to producing superposed images (at different levels), but to make 115 both images if desired at either the exterior face as in Fig. 8, or as in Fig. 9 the interior 115 face, of the colloid layer, so that in the latter case the resulting compound color image 120 is protected from abrasion on one side by the transparent carrier, and upon the other by a layer of clear gelatin. Such an image should not only be many times less subject 125 to abrasion in use than the films with images on both sides of the carrier which are now being produced and used, but even less subject to injury than the ordinary black-and-white motion picture positives printed in the usual way upon the outer face of the colloid layer.

It is worthy of note that any process depending upon the production of the second 130

image in an uneven residual layer of silver bromid has the following practical disadvantage, which is totally eliminated in my process. The residual layer is not only of uneven thickness, which is contrary to the normal condition for producing a photographic image with correct gradations, but it will vary in both thickness and unevenness according to the density and character 10 of the negative used in producing the first print, and the depth to which it is developed, thus making variable and indefinite conditions for the production of the second print; and this objection can only be minimized and not removed even by saturating the colloid layer with a nonactinic dye to limit the depth of penetration of actinic light, in accordance with my U. S. Patent 1,186,000 granted June 6, 1916. Only in 20 my present process is a second print made in silver bromid under the correct or normal conditions of exposure upon a colloid layer fully and evenly charged with sensitive silver bromid, thus securing the most favorable and definite and perfectly uniform conditions for the production of a perfect image.

This application is in part a continuation of prior application Serial No. 420,431, filed 30 October 29, 1920, the present application claiming the invention broadly, and claiming also the species in which the two images are at the same surface of the colloid layer, the other species, in which the images are at 35 the opposite surfaces, being reserved and claimed in said copending application.

It will thus be seen that a color photograph or motion picture film, also a method of producing it, have been described, which 40 embody the principles and attain the objects of the present invention. Since matters of procedure, manipulation, ingredients, arrangement, combination, and other features, may be variously modified without 45 departing from the underlying principles, it is not desired to limit the invention except in so far as specified in the appended claims.

What is claimed is:

50 1. In photographic color print making, the production of a silver image which is converted in part to silver ferrocyanid, followed by reconverting the silver ferrocyanid to silver bromid and then exposed to light under another negative and developing a second silver print which is subsequently converted into a color print.

60 2. The production of a silver image in a gelatin silver bromid layer, followed by converting the silver image to a color image by a process producing silver ferrocyanid, followed by converting the silver ferrocyanid to silver bromid, thus restoring substantially the original silver bromid content to the gelatin layer, followed by ex-

posing to light under another negative and developing a silver print which is subsequently converted to another color.

3. The production of a silver image in a gelatin bromid layer, followed by converting the silver image to a color image by a process producing silver ferrocyanid, followed by converting the silver ferrocyanid to light-sensitive silver bromid, thus substantially restoring the original evenly distributed light-sensitive silver bromid content of the gelatin layer, followed by exposing to light under another negative and developing a silver print which is subsequently converted to another color. 75

4. The production of a color image in a gelatin silver bromid layer, followed by the production of a silver image in the same layer which is not limited to an uneven residual layer of silver bromid left after the production of the first image, but is produced in a layer fully and evenly charged with light-sensitive silver bromid. 85

5. In the successive production of two different color images in a gelatin silver bromid layer, rendering the base of the first image unredevelopable without subsequent exposure to light, by reconverting it to light sensitive material, in contradistinction to dissolving it out or making it inert to light and development. 90

6. As an intermediate product in a color photography process, a gelatin silver bromid film containing a color image, but evenly charged throughout its body with light-sensitive silver bromid. 100

7. As an intermediate product in color photography process, a gelatin silver bromid film containing a color image, but evenly charged throughout its body with evenly light-sensitive silver bromid. 105

8. As an intermediate product in a color photography process, a gelatin silver bromid film containing a color image which is transparent to actinic light, but which film is also evenly charged throughout its body with light-sensitive silver bromid, and thus adapted to the production of a second image by exposure and development upon either face. 110

9. As an intermediate product in a color photography process, a gelatin silver bromid film containing a color image which is transparent to actinic light, but which film is also evenly charged throughout its body with light-sensitive silver bromid, and thus adapted to the production of a second image by exposure and development upon either face, and without limitation to an uneven residual layer of silver bromid left after the production of the first image. 120

10. As an intermediate product in a color photography process, a gelatin silver bromid film containing a color image which is transparent to actinic light, but which film is 125

also evenly charged throughout its body with light-sensitive silver-bromid, and thus adapted to the production of a second image by exposure and development upon either 5 face, and to any desired depth within the layer.

11. The production of a silver image in a gelatin silver bromid layer, followed by converting the silver image to a color image by 10 a process producing silver ferrocyanid and a color transparent to actinic light, followed by converting the silver ferrocyanid to light-sensitive silver-bromid, thus substantially restoring the original evenly distributed light- 15 sensitive silver bromid content of the gelatin layer, followed by exposure to light under another negative and upon the same face as the first print, and developing a silver print which is subsequently converted to another color, and which therefore occupies the 20 same face and level as the first print.

12. Two different color images produced successively in the same colloid layer, each 25 by exposure and development of silver bromid followed by color conversion, and both in the same face and level of the colloid layer.

13. Two different colored registered and 30 blended images buried in a single colloid layer, protected on one side by the transparent carrier and upon the other side by a covering which is part of the original colloid layer.

14. Method of producing a color photograph or film by blending differently colored images within the same colloid layer containing a silver haloid upon a suitable carrier consisting in making each of said 35 respective images by the action of light upon a silver haloid followed by development and conversion to color images, the first image being color-converted from the silver image by a process producing a ferrocyanid compound, and such compound being thereafter 40 submitted to the action of a halogen to re-sensitize the colloid layer before exposure for the second image.

15. Method of producing a color photograph or film consisting in making an 45 image by exposure of a layer sensitized with

silver bromid, developing such image, color-toning such image by a process producing silver ferrocyanid, treating the same to re-convert the silver salt to silver bromid, thus restoring sensitiveness, making a second image by exposure of the same layer, and developing and color-toning the second image. 55

16. In the process of producing two images in a single layer of colloid emulsion containing a silver haloid by successive 60 printings with intermediate development and conversion of the first image, restoring the evenness of sensitivity after the development and conversion of the first image by re-converting to sensitiveness the silver used 65 in the first image, so that the second image can be exposed and developed from a uniform emulsion to yield normal gradations.

17. In the production of color prints in a single colloid layer containing a silver 70 haloid on a transparent carrier, printing a silver image from a red record negative through the carrier, developing it as a silver image adjacent to the carrier, converting it to a pigment blue-to-green print by chemical treatment without dyeing, and subsequently producing a red image in registry 75 therewith in the same colloid layer.

18. In the production of color prints in a single colloid layer containing a silver haloid on a transparent carrier, photographically producing a silver image from a red record negative and converting it to a pigment 80 blue-to-green print by chemical treatment without dyeing, conjointly with treatment 85 with a haloid, and the subsequent production of a red image in the same colloid layer.

19. In the production of photographic multi-color prints in a single colloid layer containing a silver haloid, the production of 90 a silver image from a red record negative followed by conversion to a pigment blue-to-green print by chemical treatment without dyeing, and conjoint treatment with a haloid to prevent redevelopment of the original image together with another image subsequently produced in the same colloid layer. 95

In testimony whereof, I have affixed my signature hereto.

FREDERIC E. IVES.